

Patented Nov. 26, 1946

2,411,811

# UNITED STATES PATENT OFFICE

2,411,811

## LIGHT-SENSITIVE MATERIALS

Donald Edward Sargent, Easton, Pa., assignor to  
General Aniline & Film Corporation, New  
York, N. Y., a corporation of Delaware

No Drawing. Application February 1, 1945,  
Serial No. 575,737

18 Claims. (Cl. 95—6)

1

This invention relates to photoprinting material for the direct reproduction of positive prints from positive originals and negative prints from negative originals. More particularly, it relates to a photoprinting material comprising a light sensitive element which will decompose upon exposure to light and furnish a dye component in its undecomposed form and to the process of producing such photoprinting material.

Many processes have been suggested for the production of photoprinting material of this type, such processes differing principally in the chemical used as the light sensitive element and in the manner of developing a dye image. The most widely known of these processes are those which are based upon the light sensitivity of aromatic diazo compounds. Other such processes of less importance include processes based upon the light sensitivity of the leuco compounds of the coal tar dyestuffs; processes based upon the oxidizing action of o-nitro groups in aromatic systems having aliphatic side chains, as for instance o-nitrophenyl lactic acid methylketone; and processes based upon the light sensitivity of the o-nitro-diaminotriphenyl-methane bases. With the exception of the processes based upon the light sensitivity of aromatic diazo compounds, these suggested photoprinting processes for the reproduction of positive copies from positive originals have found no commercial adaptability either because of the instability of the compounds employed or the difficulty of developing the dye image from the undecomposed light sensitive material. The aromatic diazo compounds have found wide commercial acceptance in two well-known processes which are designated respectively as the one-component or wet-development process and the two-component or dry-development process. In the one-component process, the aromatic diazo compound is incorporated into a light sensitive layer on the carrier which may be paper, foil, glass or a metallic surface, and after exposure under the original to be copied is developed by contact with a solution of the coupling component necessary to produce the ultimately desired image. In the two-component process, the aromatic diazo compound and the coupling component necessary to produce the dye image are both incorporated in the light sensitive layer on the carrier. In this case, the development of the dye image is effected after exposure by contacting the light sensitive layer with ammonia gas. For optimum results, it is necessary to limit the selection of the diazo compound to the diazo compounds derived from aromatic p-diamines and o-aminonaphthols since premature coupling of the dye components takes place if other types of diazos are used in the light sensitive layer together with the coupling compo-

1  
2  
nent, thus reducing the keeping quality of the coated carrier.

In photoprinting processes of this type, it is highly desirable to produce a copy which will have a clear white background and which will not be subject to discoloration in the background due to aging. It is also desirable to have a material which will give gradation of shade throughout the high light and half tone areas. In the case of the aromatic diazo compounds, the light decomposition products remaining in the background will become discolored after a short time and in view of this characteristic it has been found necessary to incorporate materials which will partially inhibit or retard this tendency toward discoloration in order to maintain a reasonably acceptable clear background.

It has now been discovered that another class of compounds may be used as the light sensitive element in the preparation of positive reproduction photoprinting material which, when coated onto a suitable carrier such as the paper, foil, glass or metallic surfaces mentioned above, together with a suitable dye component will form an azo dye when developed in a proper medium and will decompose to a non-dye forming compound upon exposure to light. This class of compounds may be designated as N-nitroso-N-arylamides. These nitrosoarylamides are stable in neutral and weakly acidic media but are sensitive to both alkalies and strong acids. They may be represented by the following general formula



35  
36  
37  
38  
39  
40  
41  
42  
43  
44  
45  
46  
47  
48  
49  
50  
51  
52  
53  
54  
55  
56  
57  
58  
59  
60  
61  
62  
63  
64  
65  
66  
67  
68  
69  
70  
71  
72  
73  
74  
75  
76  
77  
78  
79  
80  
81  
82  
83  
84  
85  
86  
87  
88  
89  
90  
91  
92  
93  
94  
95  
96  
97  
98  
99  
100  
101  
102  
103  
104  
105  
106  
107  
108  
109  
110  
111  
112  
113  
114  
115  
116  
117  
118  
119  
120  
121  
122  
123  
124  
125  
126  
127  
128  
129  
130  
131  
132  
133  
134  
135  
136  
137  
138  
139  
140  
141  
142  
143  
144  
145  
146  
147  
148  
149  
150  
151  
152  
153  
154  
155  
156  
157  
158  
159  
160  
161  
162  
163  
164  
165  
166  
167  
168  
169  
170  
171  
172  
173  
174  
175  
176  
177  
178  
179  
180  
181  
182  
183  
184  
185  
186  
187  
188  
189  
190  
191  
192  
193  
194  
195  
196  
197  
198  
199  
200  
201  
202  
203  
204  
205  
206  
207  
208  
209  
210  
211  
212  
213  
214  
215  
216  
217  
218  
219  
220  
221  
222  
223  
224  
225  
226  
227  
228  
229  
230  
231  
232  
233  
234  
235  
236  
237  
238  
239  
240  
241  
242  
243  
244  
245  
246  
247  
248  
249  
250  
251  
252  
253  
254  
255  
256  
257  
258  
259  
260  
261  
262  
263  
264  
265  
266  
267  
268  
269  
270  
271  
272  
273  
274  
275  
276  
277  
278  
279  
280  
281  
282  
283  
284  
285  
286  
287  
288  
289  
290  
291  
292  
293  
294  
295  
296  
297  
298  
299  
300  
301  
302  
303  
304  
305  
306  
307  
308  
309  
310  
311  
312  
313  
314  
315  
316  
317  
318  
319  
320  
321  
322  
323  
324  
325  
326  
327  
328  
329  
330  
331  
332  
333  
334  
335  
336  
337  
338  
339  
340  
341  
342  
343  
344  
345  
346  
347  
348  
349  
350  
351  
352  
353  
354  
355  
356  
357  
358  
359  
360  
361  
362  
363  
364  
365  
366  
367  
368  
369  
370  
371  
372  
373  
374  
375  
376  
377  
378  
379  
380  
381  
382  
383  
384  
385  
386  
387  
388  
389  
390  
391  
392  
393  
394  
395  
396  
397  
398  
399  
400  
401  
402  
403  
404  
405  
406  
407  
408  
409  
410  
411  
412  
413  
414  
415  
416  
417  
418  
419  
420  
421  
422  
423  
424  
425  
426  
427  
428  
429  
430  
431  
432  
433  
434  
435  
436  
437  
438  
439  
440  
441  
442  
443  
444  
445  
446  
447  
448  
449  
450  
451  
452  
453  
454  
455  
456  
457  
458  
459  
460  
461  
462  
463  
464  
465  
466  
467  
468  
469  
470  
471  
472  
473  
474  
475  
476  
477  
478  
479  
480  
481  
482  
483  
484  
485  
486  
487  
488  
489  
490  
491  
492  
493  
494  
495  
496  
497  
498  
499  
500  
501  
502  
503  
504  
505  
506  
507  
508  
509  
510  
511  
512  
513  
514  
515  
516  
517  
518  
519  
520  
521  
522  
523  
524  
525  
526  
527  
528  
529  
530  
531  
532  
533  
534  
535  
536  
537  
538  
539  
540  
541  
542  
543  
544  
545  
546  
547  
548  
549  
550  
551  
552  
553  
554  
555  
556  
557  
558  
559  
550  
551  
552  
553  
554  
555  
556  
557  
558  
559  
560  
561  
562  
563  
564  
565  
566  
567  
568  
569  
570  
571  
572  
573  
574  
575  
576  
577  
578  
579  
580  
581  
582  
583  
584  
585  
586  
587  
588  
589  
590  
591  
592  
593  
594  
595  
596  
597  
598  
599  
600  
601  
602  
603  
604  
605  
606  
607  
608  
609  
610  
611  
612  
613  
614  
615  
616  
617  
618  
619  
620  
621  
622  
623  
624  
625  
626  
627  
628  
629  
630  
631  
632  
633  
634  
635  
636  
637  
638  
639  
640  
641  
642  
643  
644  
645  
646  
647  
648  
649  
650  
651  
652  
653  
654  
655  
656  
657  
658  
659  
660  
661  
662  
663  
664  
665  
666  
667  
668  
669  
670  
671  
672  
673  
674  
675  
676  
677  
678  
679  
680  
681  
682  
683  
684  
685  
686  
687  
688  
689  
690  
691  
692  
693  
694  
695  
696  
697  
698  
699  
700  
701  
702  
703  
704  
705  
706  
707  
708  
709  
710  
711  
712  
713  
714  
715  
716  
717  
718  
719  
720  
721  
722  
723  
724  
725  
726  
727  
728  
729  
730  
731  
732  
733  
734  
735  
736  
737  
738  
739  
740  
741  
742  
743  
744  
745  
746  
747  
748  
749  
750  
751  
752  
753  
754  
755  
756  
757  
758  
759  
750  
751  
752  
753  
754  
755  
756  
757  
758  
759  
760  
761  
762  
763  
764  
765  
766  
767  
768  
769  
770  
771  
772  
773  
774  
775  
776  
777  
778  
779  
770  
771  
772  
773  
774  
775  
776  
777  
778  
779  
780  
781  
782  
783  
784  
785  
786  
787  
788  
789  
790  
791  
792  
793  
794  
795  
796  
797  
798  
799  
800  
801  
802  
803  
804  
805  
806  
807  
808  
809  
8010  
8011  
8012  
8013  
8014  
8015  
8016  
8017  
8018  
8019  
8020  
8021  
8022  
8023  
8024  
8025  
8026  
8027  
8028  
8029  
8030  
8031  
8032  
8033  
8034  
8035  
8036  
8037  
8038  
8039  
8040  
8041  
8042  
8043  
8044  
8045  
8046  
8047  
8048  
8049  
8050  
8051  
8052  
8053  
8054  
8055  
8056  
8057  
8058  
8059  
8060  
8061  
8062  
8063  
8064  
8065  
8066  
8067  
8068  
8069  
8070  
8071  
8072  
8073  
8074  
8075  
8076  
8077  
8078  
8079  
8080  
8081  
8082  
8083  
8084  
8085  
8086  
8087  
8088  
8089  
8090  
8091  
8092  
8093  
8094  
8095  
8096  
8097  
8098  
8099  
80100  
80101  
80102  
80103  
80104  
80105  
80106  
80107  
80108  
80109  
80110  
80111  
80112  
80113  
80114  
80115  
80116  
80117  
80118  
80119  
80120  
80121  
80122  
80123  
80124  
80125  
80126  
80127  
80128  
80129  
80130  
80131  
80132  
80133  
80134  
80135  
80136  
80137  
80138  
80139  
80140  
80141  
80142  
80143  
80144  
80145  
80146  
80147  
80148  
80149  
80150  
80151  
80152  
80153  
80154  
80155  
80156  
80157  
80158  
80159  
80160  
80161  
80162  
80163  
80164  
80165  
80166  
80167  
80168  
80169  
80170  
80171  
80172  
80173  
80174  
80175  
80176  
80177  
80178  
80179  
80180  
80181  
80182  
80183  
80184  
80185  
80186  
80187  
80188  
80189  
80190  
80191  
80192  
80193  
80194  
80195  
80196  
80197  
80198  
80199  
80200  
80201  
80202  
80203  
80204  
80205  
80206  
80207  
80208  
80209  
80210  
80211  
80212  
80213  
80214  
80215  
80216  
80217  
80218  
80219  
80220  
80221  
80222  
80223  
80224  
80225  
80226  
80227  
80228  
80229  
80230  
80231  
80232  
80233  
80234  
80235  
80236  
80237  
80238  
80239  
80240  
80241  
80242  
80243  
80244  
80245  
80246  
80247  
80248  
80249  
80250  
80251  
80252  
80253  
80254  
80255  
80256  
80257  
80258  
80259  
80260  
80261  
80262  
80263  
80264  
80265  
80266  
80267  
80268  
80269  
80270  
80271  
80272  
80273  
80274  
80275  
80276  
80277  
80278  
80279  
80280  
80281  
80282  
80283  
80284  
80285  
80286  
80287  
80288  
80289  
80290  
80291  
80292  
80293  
80294  
80295  
80296  
80297  
80298  
80299  
80300  
80301  
80302  
80303  
80304  
80305  
80306  
80307  
80308  
80309  
80310  
80311  
80312  
80313  
80314  
80315  
80316  
80317  
80318  
80319  
80320  
80321  
80322  
80323  
80324  
80325  
80326  
80327  
80328  
80329  
80330  
80331  
80332  
80333  
80334  
80335  
80336  
80337  
80338  
80339  
80340  
80341  
80342  
80343  
80344  
80345  
80346  
80347  
80348  
80349  
80350  
80351  
80352  
80353  
80354  
80355  
80356  
80357  
80358  
80359  
80360  
80361  
80362  
80363  
80364  
80365  
80366  
80367  
80368  
80369  
80370  
80371  
80372  
80373  
80374  
80375  
80376  
80377  
80378  
80379  
80380  
80381  
80382  
80383  
80384  
80385  
80386  
80387  
80388  
80389  
80390  
80391  
80392  
80393  
80394  
80395  
80396  
80397  
80398  
80399  
80400  
80401  
80402  
80403  
80404  
80405  
80406  
80407  
80408  
80409  
80410  
80411  
80412  
80413  
80414  
80415  
80416  
80417  
80418  
80419  
80420  
80421  
80422  
80423  
80424  
80425  
80426  
80427  
80428  
80429  
80430  
80431  
80432  
80433  
80434  
80435  
80436  
80437  
80438  
80439  
80440  
80441  
80442  
80443  
80444  
80445  
80446  
80447  
80448  
80449  
80450  
80451  
80452  
80453  
80454  
80455  
80456  
80457  
80458  
80459  
80460  
80461  
80462  
80463  
80464  
80465  
80466  
80467  
80468  
80469  
80470  
80471  
80472  
80473  
80474  
80475  
80476  
80477  
80478  
80479  
80480  
80481  
80482  
80483  
80484  
80485  
80486  
80487  
80488  
80489  
80490  
80491  
80492  
80493  
80494  
80495  
80496  
80497  
80498  
80499  
80500  
80501  
80502  
80503  
80504  
80505  
80506  
80507  
80508  
80509  
80510  
80511  
80512  
80513  
80514  
80515  
80516  
80517  
80518  
80519  
80520  
80521  
80522  
80523  
80524  
80525  
80526  
80527  
80528  
80529  
80530  
80531  
80532  
80533  
80534  
80535  
80536  
80537  
80538  
80539  
80540  
80541  
80542  
80543  
80544  
80545  
80546  
80547  
80548  
80549  
80550  
80551  
80552  
80553  
80554  
80555  
80556  
80557  
80558  
80559  
80560  
80561  
80562  
80563  
80564  
80565  
80566  
80567  
80568  
80569  
80570  
80571  
80572  
80573  
80574  
80575  
80576  
80577  
80578  
80579  
80580  
80581  
80582  
80583  
80584  
80585  
80586  
80587  
80588  
80589  
80590  
80591  
80592  
80593  
80594  
80595  
80596  
80597  
80598  
80599  
80600  
80601  
80602  
80603  
80604  
80605  
80606  
80607  
80608  
80609  
80610  
80611  
80612  
80613  
80614  
80615  
80616  
80617  
80618  
80619  
80620  
80621  
80622  
80623  
80624  
80625  
80626  
80627  
80628  
80629  
80630  
80631  
80632  
80633  
80634  
80635  
80636  
80637  
80638  
80639  
80640  
80641  
80642  
80643  
80644  
80645  
80646  
80647  
80648  
80649  
80650  
80651  
80652  
80653  
80654  
80655  
80656  
80657  
80658  
80659  
80660  
80661  
80662  
80663  
80664  
80665  
80666  
80667  
80668  
80669  
80670  
80671  
80672  
80673  
80674  
80675  
80676  
80677  
80678  
80679  
80680  
80681  
80682  
80683  
80684  
80685  
80686  
80687  
80688  
80689  
80690  
80691  
80692  
80693  
80694  
80695  
80696  
80697  
80698  
80699  
80700  
80701  
80702  
80703  
80704  
80705  
80706  
80707  
80708  
80709  
80710  
80711  
80712  
80713  
80714  
80715  
80716  
80717  
80718  
80719  
80720  
80721  
80722  
80723  
80724  
80725  
80726  
80727  
80728  
80729  
80730  
80731  
80732  
80733  
80734  
80735  
80736  
80737  
80738  
80739  
80740  
80741  
80742  
80743  
80744  
80745  
80746  
80747  
80748  
80749  
80750  
80751  
80752  
80753  
80754  
80755  
80756  
80757  
80758  
80759  
80760  
80761  
80762  
80763  
80764  
80765  
80766  
80767  
80768  
80769  
80770  
80771  
80772  
80773  
80774  
80775  
80776  
80777  
80778  
80779  
80780  
80781  
80782  
80783  
80784  
80785  
80786  
80787  
80788  
80789  
80790  
80791  
80792  
80793  
80794  
80795  
80796  
80797  
80798  
80799  
80800  
80801  
80802  
80803  
80804  
80805  
80806  
80807  
80808  
80809  
80810  
80811  
80812  
80813  
80814  
80815  
80816  
80817  
80818  
80819  
80820  
80821  
80822  
80823  
80824  
80825  
80826  
80827  
80828  
80829  
80830  
80831  
80832  
80833  
80834  
80835  
80836  
80837  
80838  
80839  
80840  
80841  
80842  
80843  
80844  
80845  
80846  
80847  
80848  
80849  
80850  
80851  
80852  
80853  
80854  
80855  
80856  
80857  
80858  
80859  
80860  
80861  
80862  
80863  
80864  
80865  
80866  
80867  
80868  
80869  
80870  
80871  
80872  
80873  
8

It is this hydrolysis product or aryl diazotate salt which is utilized to produce the azo dye image by coupling with an azo coupling component and hence the treatment of an N-nitroso-N-arylamide with an alkali in the presence of an azo coupling component will produce a dye. These N-nitroso-N-arylamides are also altered by treatment with a strong acid such as hydrochloric acid, the end product in that case being a diazonium salt. Specifically, it is presumed to follow the following reactions:



As is indicated above, a light sensitive material to be suitable for positive photoprinting purposes in a practical sense must be capable of forming a dye image upon development with another dye component and in the case of two-component layers, the light sensitive material must be such that it will not readily couple with the other dye component in the absence of the coupling medium. Preferably it should be incapable of coupling in the absence of a coupling medium. In addition, the light sensitive material must be decomposable to a compound which will no longer perform the dye function. This is necessary in order to insure the absence of color in the high light areas or in the areas which are exposed to light by reason of the absence of lines or figures in the original which otherwise would prevent the passage of light through the original. The N-nitroso-N-arylamides of this invention, as indicated in the above equations, will couple with an azo coupling component to form a dye in the presence of an alkaline medium. They are stable and will not couple with an azo coupling component in the absence of an alkali. As indicated above, the N-nitroso-N-arylamides are altered to diazonium salts by strong acids. However, they are not changed by weak acids and are particularly stable in solution having a pH of from about 5 to 7. Furthermore, it has now been found that they are sufficiently light sensitive to form the basis of a positive photoprinting material and that upon exposure to light they will decompose to products which will no longer couple to form a dye. It has also been found that the light decomposition products of the N-nitroso-N-arylamides do not readily couple with residual undecomposed N-nitroso-N-arylamide compounds and do not otherwise contribute to the formation of discoloration in the exposed areas of the reproduction. Thus, the white areas of the reproduction remain white for long periods of time and do not become discolored except by possible aging of the paper or other carrier employed in the production of the photoprinting material.

In its preferred embodiment, the process of this invention is carried out by coating a suitable base such as paper, a cellulose or cellulose ester film, glass plate, textile material, gelatinized surface or metallic surface with a coating preparation containing an N-nitroso-N-arylamide compound, an azo coupling component such as a phenolic substance or a compound having an active methylene group, a mild acid such as citric or acetic acid and water. The coating is effected in the usual manner by applying the coating solution to the surface of the carrier or base material with a doctor blade or by spraying. The coated material is then dried, exposed under

an original positive or negative picture or drawing and developed by treatment with ammonia vapor or other suitable alkaline materials. As the diluent for the coating solution, organic solvents of high volatility, such as alcohols, ethers, and ketones, as for example, acetone, may be employed in place of water. Such diluents may be employed to make up the nitrosoamide and coupler coating solution in cases where the base material or carrier is such that it will resist the penetrating and solvent action of the diluent. High temperature drying may thus be avoided.

In another manner of carrying out this process only the N-nitroso-N-arylamide compound is added to the mild acid solution and coated onto the carrier. The exposure under a suitable positive is effected as before but the image is developed by bathing the exposed element in an alkaline bath containing the azo dye coupler necessary to combine with the undecomposed nitrosoamide compound to form a dye in the unexposed areas. In this modification of the process, it is desirable, although not necessary, to employ a non-migratory N-nitroso-N-arylamide such as N-nitroso-N-phenylstearamide in order to prevent diffusion of the image in the developing bath.

In still another manner of operating the process of this invention N-nitroso-N-arylamides may be used which have the property of self-coupling under the influence of alkalis to produce colors. An example of such a compound is N-nitroso-N-phenyl-N'-β-naphthylurea,



Here the self-coupling nitrosoamide is added to mildly acid aqueous solution and coated onto a suitable carrier in the usual manner. It is then exposed to a suitable source of light under a positive and developed by merely contacting the unexposed areas with ammonia vapor or a solution of an alkaline compound. This alkaline developing treatment produces the necessary rearrangement in the nitrosoamide molecule to produce the chromophore group and at the same time effects the coupling of the thus rearranged molecule with a degradation product of the nitrosoamide compound. It is believed that the nitrosoamide after rearrangement couples with the naphthyl amine fragment resulting from rearrangement hydrolysis, and decarboxylation which is presumed to take place in accordance with the following scheme:



in the specific instance of the N-nitroso-N-phenyl-N'- $\beta$ -naphthyl-urea, the image is developed to a brownish orange color.

Although it is not essential, it is understood that, if desired, auxiliary materials may be added to the coating solution in any of the modifications of this process which materials may function as stabilizers, preservatives, extenders, color intensifiers, and light sensitive intensifiers.

A wide range of colors may be produced by this process. By proper selection of the coupling component the N-nitroso-N-arylamide light sensitive layers can be made to reproduce the image in almost any desired color. Suitable coupling components for this purpose include resorcylic acid, phenol, resorcinol, chromotrope acid, 2,3-dihydroxynaphthalene, H-acid, R-salt, 2-hydroxy-1-benzene-sulfonic acid, 2,5-dimethyl-6- $\omega$ -dimethyl-aminomethyl-1-phenol, the aminomethylamide of 2,3-hydroxynaphthoic acid, phloroglucin, 2,3-dihydroxy-naphthalene-monoxyethylether, and  $\beta$ -naphthol-3,6-disulfonic acid.

The N-nitroso-N-arylamides of this invention are most sensitive to light waves in the violet and ultraviolet range. Consequently, any source of light such as a quartz mercury vapor arc lamp which emits rays in that region may be employed for exposing the light sensitive layer for the purpose of decomposing the N-nitroso-N-arylamide in the high light areas. Other sources of light which may be employed include incandescent lamps, arc lamps, and fluorescent lamps. However, the process is not necessarily restricted to the frequencies of the violet and near ultraviolet range since the sensitivity of the nitrosoamides could be adjusted to permit the absorption of other frequencies such as those in the red and blue ranges.

The practice of this invention may be best understood by reference to the following specific examples which are presented as illustrative of the process involved and without any intention of introducing limitations. Unless otherwise stated, the parts given are by weight.

#### Example 1

A solution was made up containing 5 parts of p-methoxy-phenylurea, and 50 parts of glacial acetic acid.

This solution was treated with a concentrated aqueous solution of sodium nitrite until nitrosation was complete.

The resulting solution of N-nitroso-N-(p-methoxyphenyl)-urea was then added while stirring to a solution containing 10 parts of chromotrope acid (1,8-dihydroxynaphthalene-3,6-disulfonic acid) in 500 parts of water.

This mixture was coated onto a paper strip and dried. The coated paper strip was then exposed under a positive to the light from a quartz mercury vapor arc lamp. The positive original was removed and the exposed coated paper developed by inserting it in a chamber filled with ammonia fumes. The image on the original was developed as a positive magenta colored print having a clear white background. In this example, if the 10 parts of chromotrope acid be replaced by 10 parts of 2,3-dihydroxynaphthalene the original will be reproduced in a dark blue image.

#### Example 2

A solution containing 5 parts of p-diethylaminophenyl-urea and 50 parts of glacial acetic acid was treated with a concentrated aqueous

solution of sodium nitrite until nitrosation was complete.

The N-nitroso-N-(p-diethylaminophenyl)-urea obtained from this nitrosation was added to a solution containing 10 parts of resorcylic acid and 50 parts of water.

This mixture was coated onto a paper strip and dried. It was then exposed to light from a 100 w. incandescent lamp under a positive original for 10 minutes and the image developed by inserting the exposed coated paper into a chamber containing ammonia fumes. The design of the positive original was developed to a black-maroon positive image having a clear white background. In this example if the 10 parts of resorcylic acid be replaced by 10 parts of phenol, the original will be reproduced in a yellow dye image. The time of exposure may be reduced considerably by substituting a lamp of higher efficiency, such as a "G. E. 360 BL" lamp for the 100 w. lamp.

#### Example 3

A solution containing 5 parts of p-phenylenediamine in 50 parts of glacial acetic acid was treated with one equivalent of sodium nitrite (about 1.7 parts) dissolved in a small amount of water. The resulting solution of nitrosoamide was added to a solution containing 10 parts of H-acid (8-amino-1-naphthol-3,6-disulfonic acid) in 500 parts of water.

The resulting mixture was coated onto a paper strip and allowed to dry in the dark. It was then exposed to light under a positive transparency and the exposed coated paper developed by contacting same with ammonia vapor. The design of the positive transparency was developed to a purple positive dye image on a clear white background.

#### Example 4

A solution containing 5 parts of N-nitroso-N-phenyl-N'- $\beta$ -naphthylurea obtained by oxidizing 2-phenyl-4- $\beta$ -naphthylsemicarbazide and 50 parts of glacial acetic acid was added to 500 parts of water and the resulting mixture coated on strips of paper, cloth, and gelatinized glass plates and dried in the dark.

The dried coated strips of paper, cloth, and gelatinized glass were each exposed to light under a positive transparency and the thus exposed elements developed by contracting same with ammonia gas, the images in each case were developed to a brownish orange color on a clear background.

#### Example 5

An acetic acid solution of N-nitroso-N-phenylstearamide prepared by nitrosation of N-phenylstearamide with nitrous fumes in glacial acetic acid was coated onto a textile base and allowed to dry in the dark. The dried coated textile was then exposed to a proper source of light under a stencil. It was then placed in a solution containing 10 parts of R-salt (2-naphthol-3,6-disulfonic acid) and 20 parts of sodium carbonate in 500 parts of water.

It was then washed and dried. A very excellent printed textile was thus obtained having the design of the stencil reproduced in a bright red color on a clear background.

Having now set forth and fully described my invention, and having illustrated the best manner to perform it, what I desire to protect by Letters Patent and, therefore, claim is:

1. The process of producing a photoprinting material which comprises coating a solution of a

light-sensitive N-nitroso-N-arylamide onto a suitable carrier and drying.

2. The process of producing a photoprinting material which comprises coating a solution comprising a light-sensitive N-nitroso-N-arylamide and an azo coupling component onto a suitable carrier and drying.

3. The process of producing a photoprinting material which comprises incorporating a light-sensitive N-nitroso-N-arylamide and an azo coupling component into a weakly acid aqueous solution, coating the resulting solution onto a suitable carrier and drying.

4. The process of producing a photoprinting material which comprises incorporating N-nitroso-N-(p-diethylaminophenyl)-urea and an azo coupling component into a weakly acid aqueous solution, coating the resulting solution onto a suitable carrier and drying.

5. The process of producing a photoprinting material which comprises incorporating N-nitroso-N-phenylstearamide and an azo coupling component into a weakly acid aqueous solution, coating the resulting solution onto a suitable carrier and drying.

6. The process of producing a photoprinting material which comprises coating a solution of N-nitroso-N-phenyl-N'- $\beta$ -naphthylurea in weak acetic acid onto a suitable carrier and drying.

7. Photoprinting materials comprising as the light sensitive element a light-sensitive N-nitroso-N-arylamide compound.

8. Photoprinting materials comprising in combination a light-sensitive N-nitroso-N-arylamide compound as the light sensitive element and an azo coupling component.

9. Photoprinting materials comprising a light sensitive layer on a suitable carrier, said light sensitive layer containing a light-sensitive N-nitroso-N-arylamide as the light sensitive element.

10. Photoprinting materials comprising a light sensitive layer on a suitable carrier, said light sensitive layer containing an N-nitroso-N-arylamide as the light sensitive element and an azo coupling component.

11. Photoprinting materials comprising a light sensitive layer on a suitable carrier, said light sensitive layer containing N-nitroso-N-(p-diethylaminophenyl)-urea as the light sensitive element and an azo coupling component.

12. Photoprinting materials comprising a light sensitive layer on a suitable carrier, said light sensitive layer containing N-nitroso-N-phenylstearamide as the light sensitive element and an azo coupling component.

13. Photoprinting materials comprising a light sensitive layer on a suitable carrier, said light

sensitive layer containing N-nitroso-N-phenyl-N'- $\beta$ -naphthylurea as the light sensitive element.

14. The process of reproducing an original in its photographically positive image which comprises placing the original in contact with a photoprinting material consisting of a carrier having a light sensitive layer in which the light sensitive element is a light-sensitive N-nitroso-N-arylamide, exposing to light, and developing the image on the photoprinting material by contacting it with a developing agent selected from the group consisting of alkalis and strong acids in the presence of an azo dye coupling component.

15. The process of reproducing an original in its photographically positive image which comprises placing the original under a photoprinting material consisting of a carrier having a light sensitive layer which contains as the light sensitive element a light-sensitive N-nitroso-N-arylamide and an azo dye coupling component, exposing the photoprinting material to light through the original and developing the image of the original of the photoprinting material by contacting it with ammonia fumes.

16. The process of reproducing an original in its photographically positive image which comprises placing the original under a photoprinting material consisting of a carrier having a light sensitive layer containing N-nitroso-N-(p-diethylaminophenyl)-urea as the light sensitive element and an azo dye coupling component, exposing the photoprinting material to light through the original, and developing the image of the original on the photoprinting material by contacting it with ammonia fumes.

17. The process of reproducing an original in its photographically positive image which comprises placing the original under a photoprinting material consisting of a carrier having a light sensitive layer containing N-nitroso-N-phenylstearamide as the light sensitive element, exposing the photoprinting material to light through the original, and developing the image of the original on the photoprinting material by treating it with an alkaline solution of an azo dye coupling component.

18. The process of reproducing an original in its photographically positive image which comprises placing the original under a photoprinting material consisting of a carrier having a light sensitive layer containing N-nitroso-N-phenyl-N'- $\beta$ -naphthylurea as the light sensitive element, exposing the photoprinting material to light through the original, and developing the image of the original on the photoprinting material by contacting it with ammonia fumes.

DONALD EDWARD SARGENT.